

Aug. 23, 1960

E. E. JOINER ET AL

2,949,684

HEELS WITH NAIL-HOLDING FILLERS

Filed Dec. 31, 1958



Fig. 2



Inventors  
Edgar E. Joiner  
John P. Szumski  
By their Attorney

Benjamin C. Pollard

1

2,949,684

## HEELS WITH NAIL-HOLDING FILLERS

Edgar E. Joiner, Andover, and John P. Szumski, Marblehead, Mass., assignors to Fred W. Mears Heel Company, Inc., Lawrence, Mass., a corporation of Massachusetts

Filed Dec. 31, 1958, Ser. No. 784,159

3 Claims. (Cl. 36—40)

This invention relates to a light-weight rigid heel with a nail-holding filler.

The fashion-dictated high thin heels for women's shoes have necessitated the use of strong rigid materials which do not break easily, such as rigid plastic or light-weight metals. Metal is not nailable and heretofore awkward and expensive procedures have been required for attaching metal heels. Serious problems arise also in effecting attachment of solid plastic heels by nailing.

It has been proposed to provide the plastic heels with wooden inserts for heel attaching with nails. The proposals have relied on a force fitted or adhesively bonded plug or on molding the heel material around the insert to embed it. In these structures it was necessary to use a wooden insert or plug extending well outside of the heel attaching nailing pattern since the surrounding plastic would not hold nails. Moreover, accurately sized inserts were required for inserts to be force fitted or adhesively secured in preformed heels.

It is an object of the present invention to provide a novel light-weight heel with a heel-seat engaging surface which permits a shoe upper to be easily and firmly attached by nails or screws.

According to the present invention, a heel member of light-weight rigid material in the shape of a heel but having a cavity in the heel seat engaging portion is provided with a nailable insert which is held in fixed position in the heel-seat engaging surface and in spaced relationship to the walls of the recess by a hard, nailable adhesive resinous composition. A satisfactory bond is thereby provided between the interior wall of the heel and the insert. The hardened combination of the insert and resinous composition is machineable for shaping to the contour of a shoe upper and accepts and holds nails used in heel attaching. In another aspect of the invention, the heel is provided with a nailable attaching surface provided by the adhesive resin composition alone.

The invention may be better understood with reference to the accompanying drawings, in which

Fig. 1 is an exploded view in perspective with parts broken away of the heel seat end of a shoe upper and a heel; and

Fig. 2 is a perspective view of a nailable insert which may be used in the heel of the present invention.

The heel member 10 as shown in Fig. 1 is formed with a cavity 12 in its upper portion which is filled with a nailable body 14 held centered in the cavity 12 by a resinous mass 16 adhering to the walls 18 along the sides 20 and back 22 of the cavity 12. In the heel 10 the cavity 12 is generally wedge shaped and is defined by a cavity base surface 24 which may be substantially flat, extending from the heel breast 26 to a short distance from the exterior surface of the heel at the sides 20 and back 22. Portions of the heel member 10 above this cavity base surface 24 are reduced to a shell or wall 18 which may be of substantially uniform thickness or may be provided with reinforcing thickened portions, such as the ribs 28

2

extending along the interior faces of the wall 18 parallel to the cavity base surface 24. The rim or upper edge 30 of the wall 18 is preferably relatively thin, particularly where the heel member is made of a metal, in order to simplify concaving problems.

Considerable variation is permissible in the shape and size of the cavity 12 subject to the limitation that the cavity must have a minimum outline at least slightly larger than the heel-attaching nailing pattern 32 of the shoe upper 34 with which the heel is to be used, as shown also in Fig. 1. Also the depth of the cavity 12 within this outline must be great enough to receive the portions of the heel attaching nails 36 projecting through the heel seat 38 of the shoe upper 34 in the predetermined pattern corresponding to that shown at 32 on the exposed top cross section 40 of the insert 14. It is also important that the walls 18 of the heel member surrounding the cavity 12, that is, the material of the heel member between the interior walls of the cavity and the exterior of the heel member have sufficient thickness to withstand the stresses imposed on the heel when attached to a shoe.

The heel member 10 is made in the desired heel style from a light-weight but rigid material which may be a rigid plastic, such as cellulose acetate butyrate, cellulose acetate, nylon, styrene, or acrylate resin, or a cast light-weight metal, such as aluminum or magnesium. The nailable body 14 is held in fixed position in the heel cavity 12 in spaced relation to the walls of the cavity 12 by a resinous mixture 16 comprising a thermosetting resin, a curing agent for the resin, and a selected inert material which is filler and thickener for the resin. This composition, when cured, is adhesive to both the nailable body 14 and the metal or plastic surfaces of the heel member 10, and is hard enough to be machineable. It also may be compressed sufficiently by the entering nails to retain them without splintering, since the resin material does not sufficiently penetrate the individual particles of filler to render them rigid.

The curing type resin used for the present invention is strongly adhesive to both the nailable body 14 and the metal or plastic of the heel member 10 and possesses a cured strength which will endure future machining. A preferred thermosetting resin is a polyepoxide resin (fluid at room temperature) which is a resinous glycidyl polyether of a member of a group consisting of polyhydric phenols, polyhydric alcohols and mixtures of these. The polyepoxides are complex resinous materials and may be produced by the reaction of polyhydric phenols with a polyfunctional chlorohydrin such as epichlorohydrin and glycerol chlorohydrin. The preparation of epoxide resin is shown in United States Letters Patent No. 2,506,486 to Bender et al., granted May 2, 1950, and No. 2,589,245 to Greenlee, granted March 18, 1952.

The preferred epoxide resins used in the present invention are those liquid at room temperature, to facilitate mixing, with a viscosity at 25° C. of from about 3600 to 15,000 c.p.s. However, normally solid epoxides, which may be liquefied by gentle heating, may be used. The range of epoxy equivalents is from about 170 to 210, and the molecular weight is between 340 and 400. Such epoxy resins are commercially available as Epon 820 and 828, made by the Chemical Division, Shell Oil Co. and Araldite 6005, made by the Ciba Co., Inc.

The curing agent for the epoxide resin is preferably a fluid polyamide resin, but other curing agents, such as amines, may be used with the addition of a flexibilizer or a plasticizer. Useful polyamides for combination with the epoxy resin are the products obtained by reacting polymerized polyene fat acids or their amide forming derivatives, such as their monohydric alcohol esters or their anhydrides or acyl halides, with an organic aliphatic compound possessing at least two primary amino

groups. The polymeric fat acids may be those formed for example by thermal polymerization of drying or semi-drying type fatty oils containing glycerides of polymerizable fat acids such as soybean oil, linseed oil, cottonseed oil, perilla oil, dehydrated castor oil and the like. The polymeric glyceride may then be isolated as by distillation and converted to polymeric fat acid by hydrolysis.

The polymerized fat acids, esters or anhydrides are combined with preferably equimolecular amounts of amino compounds such as ethylene diamine, diethylene triamine, hexamethylene diamine, tetraethylene pentamine or other alkylene polyamines, or mixtures of these with each other or with related compounds such as monoethanolamine. The combination reaction is brought about by heating the mixed materials at such a temperature that polyaminolysis of the fat esters or dehydration of the polyamine salts of the fat acids will occur readily. Temperatures of 150-175° C. for a few hours with an increase to 175°-225° C. for 20 to 40 minutes just prior to removal of polyamide from the reaction chamber are sufficient. The time and temperature will vary depending on the materials used and the type of product desired. Details of this resin forming process may be found in United States patent to Cowan et al. 2,450,940 of October 12, 1948. Such a polyamide resin is Versamid 125, a product of the General Mills Chemical Division.

When fluid polyamide resins are blended with liquid epoxy resins the reaction between the amino groups of the amides and the epoxy groups of the epoxies results in a three-dimensional polymer on completion of the reaction.

The ratio of epoxy to polyamide is adjusted to produce a composition adhesive but not too brittle. This is best obtained with a ratio by weight of from 50 epoxy to 50 polyamide to 60 epoxy to 40 polyamide. However, a wider range from 40 to 70 epoxy to 60 to 30 polyamide may be used. Too much epoxy yields a product too brittle; on the other hand, too high a percentage of polyamide makes a rubbery mixture.

The primary filler, which also acts as a thickening agent for the resin, may be selected from a variety of inert compressible fibrous materials, such as wood flour or ground walnut shells. Usable material for the primary filler should have a bulk volume not over 3.9 ccs./gm., and it is preferred to be about 2.3 ccs./gm. A preferred filler is BNB-100, Solka Floc, an  $\alpha$ -cellulose product from the Brown Company. It has a fineness of 100 mesh.

The primary filler, such as the wood flour, is used to the extent of from about 10 to about 35 parts by weight based on the weight of the resin, but the preferred percent is about 15 to 25 parts by weight based on the weight of the resin. The upper limit is determined by the difficulty in molding.

If it is desired to modify the hardness or strength of the composition for reinforcement purposes, there may be added in addition small amounts of mineral fillers, i.e., up to 10% by weight, based on the weight of resin used.

The combination of filler and resin, particularly if it is to be used without the addition of a wood insert, should be selected so that the filler is not permeable to the resin, i.e., does not have its pores filled by the resin. This preserves to some extent the compressive quality of wood itself, which allows attaching nails or screws to be gripped by the penetrated surface.

The nailable insert 14 is preferably of wood but other nailable materials such as compressed fiber blocks may be used. The insert has an upper face 40 of suitable size and shape to receive heel attaching nails 36 in a predetermined pattern, and also has a depth sufficient to accept portions of the nails extending through the heel seat 38 of a shoe upper 34 in the nail pattern 32.

The over-all dimension of the insert 14 must also be small enough to allow the insert to fit within the cavity 12 with its side walls in spaced relationship to the walls 18 of the heel member 10, the space between the walls and insert being filled with the nailable resinous mixture. It is to be observed that by reason of the nailable character of the mixture in the spaces and the strong bond between the mixture and both the insert and the walls of the heel member, the minimum dimensions of the insert are not critical, although the insert does have greater nail holding power than the resinous mixture.

The hardwood insert 14, shown in Fig. 3, is conveniently prepared by cutting to size from a 1 $\frac{1}{8}$ " diameter dowel, preferably of maple. Depending upon the size of the heel, the over-all length may vary from 1 $\frac{1}{4}$ " to 1 $\frac{1}{2}$ ". One end 42 is cut perpendicular to the dowel length; the other is cut at an angle selected so that the face 40 of the insert, when in position, is generally in line with the rim 30 of the heel seat, for instance, at an angle of about 45°. The angle of the wood grain provides optimum nail holding ability and minimum danger of splitting.

A predetermined amount of moldable resin mixture 16 is deposited in the cavity 12 of the heel form 10. The wood insert 14 is centered and pressed into the resin mixture 16, forcing it down into the cavity 12 of the heel 10 to surround the insert 14 up to the level of the rim 30.

It is to be understood that the resin filler 16 may be used without the wood block insert by filling the cavity 12 of the heel 10 so that the surface at the attaching face 44 is level with the heel rim 30.

After the heel is filled with the resinous mixture or the combination resinous mixture and dowel insert, the resin is allowed to cure at room temperature overnight. Alternatively, a rapid cure may be effected by heating the freshly assembled heel shell and filler at a temperature of 190° F. for one hour.

After curing and cooling, the resinous mixture 16 is hard and firm and strongly adhesive to the walls of the heel 10. The wood insert 14 is held firmly in position. The hard filler combination is then machined by conventional procedure to a concave surface suitable for attachment to a shoe upper.

The following examples are given to aid in understanding the present invention. It is to be understood that the invention is not limited to the specific composition and procedure here described:

#### Example 1

|                                           | Parts by weight |
|-------------------------------------------|-----------------|
| Epoxide resin (Epon 820)                  | 454             |
| Polyamide resin (Versamid 125)            | 303             |
| Wood flock, 100 mesh (Solka Floc BNB-100) | 151             |

The epoxide resin was a glycidyl polyether liquid at room temperature with viscosity at 25° C. of 4,000 cps. to 14,000 cps., and an average molecular weight of 350 to 400. Reactivity range of epoxy equivalents are 175 to 210.

The polyamide resin was also fluid at room temperature with a viscosity, measured by a Brookfield viscometer, #6 spindle 4 r.p.m., at 40° C., of 80 to 120 poises and at 23° C. of 500 to 550 poises and a specific gravity of 0.97. It had an amine value ranging from 290 to 320.

The filler used was an  $\alpha$ -cellulose wood flock of 100 mesh.

The polyamide resin was added to the fluid epoxide resin and the combination was quickly and thoroughly mixed. With continued stirring, the wood flour was slowly and evenly added, the mixture increasingly thickening.

This putty-like mixture was spread in the cavity 12 in the heel-seat face 44 of a thin, high aluminum heel 10, evenly supported. A maple wood block 14 with a bottom 42, a long side 46, and the face 40 cut at an angle of

44°, was centered and pushed evenly into the soft resin mixture 16, the block-face 40 being held parallel with the heel-seat face 44, and the edge 48 extending into the cavity 12 toward the back 22 of the heel. The face 40 of the block 14 was exposed so that the front end 50 was toward the heel breast 26 and the top edge 52 toward the top back 54 of the heel 10. The resin mixture 16 was forced down toward the bottom of the cavity 12 and the top surface of the mixture rose even with the rim 30 of the heel.

The supported shell with its combination filler was put aside to cure overnight at room temperature.

The cured heel was a unitary structure with the cured resin mixture 16 firmly holding the wood block 14 centered in the heel face 44, and strongly united in turn to the walls of the cavity 12 in the heel. The attaching face of the heel, composed of the resin and embedded block, was concaved by conventional machinery for cooperation with the heel seat of a shoe upper.

The finished heel was easily and firmly attached to the corresponding upper by nailing into the face 44 of the wood insert 14 in a definite pattern 32, as shown. The nails 36 extended through the heel seat engaging face 38 of the overlasted shoe upper 34 and penetrated through the face 40 of the insert 14. The combination filler had an excellent holding power of 173 pounds.

#### Example 2

A similar aluminum heel 10 was filled with the resin mixture until the mixture was level with the heel rim 30, the wood insert being omitted. After curing, the composition was concaved. When nails were used in joining heel to upper, the resin composition was found to have nearly the same holding power.

It is to be understood that this invention is not limited to any particular style, size or shape of heel and may be employed for a heel shell of other rigid material than the metal heel shell herein described.

Having thus described our invention, what we claim as new and desire to secure by Letters Patent of the United States is:

1. A heel for a shoe comprising a rigid lightweight heel member having its upper portion formed with a cavity of an area and depth to receive portions of heel attaching nails extending through the heel seat of a shoe in the heel attaching nailing pattern, said cavity being defined by walls flaring outwardly and terminating in relatively thin upper edges, leaving the top of said heel unobstructed to receive heel attaching nails over substantially its entire area, an insert of nailable material shaped to fit within said cavity having an upper face of size and shape to extend outside said heel attaching nailing pattern to receive and hold heel attaching nails, and a body of cured hard nailable resinous composition filling spaces between the walls of said cavity and said insert, and serving as the exclusive means to hold said insert in fixed relationship to

the walls of said cavity, and the exposed surfaces of said curved resinous composition and said insert having a shape to fit against the heel seat of a corresponding shoe upper.

2. A heel for a shoe comprising a rigid lightweight metal heel member having its upper portion formed with a cavity of an area and depth to receive portions of heel attaching nails extending through the heel seat of a shoe in the heel attaching nailing pattern, said cavity being defined by walls flaring outwardly and terminating in relatively thin upper edges, leaving the top of said heel unobstructed to receive heel attaching nails over substantially its entire area, a wood insert shaped to fit within said cavity, said insert having an upper face cut at an angle of approximately 45° to the grain of said wood, and of size and shape to extend outside said heel attaching nailing pattern to receive and hold heel attaching nails, and a body of cured hard nailable resinous composition comprising a mixture of a cured thermosetting resin and a compressible fibrous material filling spaces between the walls of said cavity and said wood insert, and serving as the exclusive means to hold said insert in fixed relationship to the walls of said cavity, and the exposed surfaces of said cured resinous composition and said wood insert having a shape to fit against the heel seat of a corresponding shoe upper.

3. A heel for a shoe comprising a rigid lightweight metal heel member having its upper portion formed with a cavity of an area and depth to receive portions of heel attaching nails extending through the heel seat of a shoe in the heel attaching nailing pattern, said cavity being defined by walls flaring outwardly and terminating in relatively thin upper edges, leaving the top of said heel unobstructed to receive heel attaching nails over substantially its entire area, a wood insert shaped to fit within said cavity, said insert having an upper face cut at an angle of approximately 45° to the grain of said wood and of size and shape to extend outside said heel attaching nailing pattern to receive and hold heel attaching nails, and a body of a cured mixture of an epoxide resin and wood flour filling spaces between the walls of said cavity and said insert, and serving as the exclusive means to hold said wood insert in fixed relationship to the walls of said cavity, and the exposed surfaces of said cured resinous body and said wood insert having a shape to fit against the heel seat of a corresponding shoe upper.

#### References Cited in the file of this patent

##### UNITED STATES PATENTS

|           |         |               |
|-----------|---------|---------------|
| 1,336,194 | Burger  | Apr. 6, 1920  |
| 1,609,918 | Perugia | Dec. 7, 1926  |
| 1,710,378 | Owen    | Apr. 23, 1929 |
| 1,781,931 | Owen    | Nov. 18, 1930 |
| 2,871,583 | Cooper  | Feb. 3, 1959  |

##### FOREIGN PATENTS

|         |               |             |
|---------|---------------|-------------|
| 484,627 | Great Britain | May 9, 1938 |
|---------|---------------|-------------|